

No. 717,840.

PATENTED JAN. 6, 1903.

H. GOLDSCHMIDT.  
PROCESS OF JOINING METAL PIECES.

APPLICATION FILED JUNE 19, 1901.

NO MODEL.

2 SHEETS—SHEET 1.



Witnesses:

*Carl Bieß.  
Joh. Rohr.*

Inventor:  
Hans Goldschmidt.  
by *Kaufm. Dr. L. Goldschmidt*

Attorney.

No. 717,840.

PATENTED JAN. 6, 1903.

H. GOLDSCHMIDT.  
PROCESS OF JOINING METAL PIECES.

APPLICATION FILED JUNE 19, 1901.

NO MODEL.

2 SHEETS—SHEET 2.

Fig. 7



Fig. 8



Fig. 9.



Fig. 10.



Witnesses

Emil Hauser.

Paul Wollenberg.

Inventor  
Hans Goldschmidt.  
by Peter Steyer  
Attorney.

# UNITED STATES PATENT OFFICE.

HANS GOLDSCHMIDT, OF ESSEN-ON-THE-RUHR, GERMANY, ASSIGNOR TO  
CLARENCE B. SCHULTZ, OF BERLIN, GERMANY.

## PROCESS OF JOINING METAL PIECES.

SPECIFICATION forming part of Letters Patent No. 717,840, dated January 6, 1903.

Application filed June 19, 1901. Serial No. 65,192. (No model.)

To all whom it may concern:

Be it known that I, HANS GOLDSCHMIDT, a subject of the King of Prussia, German Emperor, and a resident of Essen-on-the-Ruhr, 5 Germany, have invented a new and Improved Process of Joining Metal Pieces, of which the following is an exact specification.

My invention relates to a new and improved process for joining metal pieces. In the processes known up to date for joining metal pieces by welding the same with the aid of the heat produced by the chemical reaction between aluminium and oxids of metals or other oxygen-containing metal compounds 15 (especially oxide of iron) the reaction mass is used only as calorifying agent and the metal produced by the reaction serves only as a heat-conductor. Therefore in these alumino-thermo processes care was taken that the molten alumina-slag at first came in contact with the pieces to be welded and only after the same had formed a protecting-coating around the pieces the molten metal was flown around the welding-pieces. In the most cases this succession took place already by the mere casting 25 of the reaction mass out of the crucible or melting-pot, as naturally at first the alumina floating above flows out and afterward the metal. Hereby it was avoided that the molten metal could come in direct contact with the molten pieces to be welded and that this metal could join with the metal pieces.

By my new process it is attained that the molten metal comes directly in contact with 35 the welding-pieces, so that the metal may partly join with the pieces, thereby strengthening the joints, whereafter the whole reaction mass begins its operation as calorifying agent for the welding process.

40 The process shall be described, for example, as used for joining rails or the like.

The joining faces of the rails are at first surrounded with a suitable mold manufactured of iron-sheet, clay, or the like, whereafter a crucible provided with a tap-hole is placed over this mold in that way that the stream of the molten mass flowing out of this hole does not directly flow upon the rails, but flows into the space between the rails and the 45 wall of the mold. Then this crucible after

closing the tap-hole is filled with the reaction mixture—for instance, a mixture of aluminium and oxide of iron—whereafter the reaction is introduced. Once the reaction being in progress further quantities of the mixture 55 may be added. When the whole mass is in reaction, the tap-hole is opened, so that at first the molten highly-overheated iron, and afterward the molten alumina floating above the iron, flows into the mold. The iron forms 60 a layer around the lower flange of the rails and effects the joining of the touching faces on this lower part. The alumina flowing out after the iron has a double effect upon the pieces to be joined. First, the heating at- 65 tained by the same may effect the welding of the joining faces; secondly, the heating of the upper part of the rails prevents the bending up of the rails near the joining faces, which bending up was tried to be done away 70 with until now in similar processes by holding the joining faces down by means of clamps and the like.

The tap-hole of the crucible may be closed by means of a clay plug or the like, or the 75 hole may be covered with a metal sheet, (iron-sheet,) asbestos, or the like before filling the crucible with the mixture. In this case the molten iron as soon as the reaction has come to the bottom of the crucible will melt this 80 covering, whereby the tap-hole will be opened automatically.

In order to make my invention more clear, I will proceed to illustrate the process by an example described at the hand of the accompanying drawings, in which similar letters denote similar parts, and in which—

Figure 1 shows a section through one of the two rails to be joined and the mold. Fig. 2 is a side view of the rails. Fig. 3 is a perspective view of the joint. Figs. 4, 5, 6, 7, 8, 9, and 10 are modified forms of arrangements for carrying the process into effect.

In Figs. 1 and 2, *a a* are the rails to be joined. *b b'* are iron-sheet molds, the upper 90 one of which consists of two parts surrounding the rails near the joining faces. The side walls *c c'* of these molds may advantageously be formed of sand or wet clay. By the special construction of the molds three hollow 95

spaces  $f f'$   $k$  are formed, in which the molten mass is cast.

The process is carried out in the following manner: The metal pieces are pressed against each other in such a manner that a displacement during the heating of the pieces by means of the reaction mass is rendered impossible. Then a crucible is filled with a mixture of aluminium and oxid of iron, both in pulverized form, whereafter the mixture is inflamed. It is advantageous to fill the crucible beforehand with a small quantity of the mixture, then to inflame the same and gradually add further quantities. When the whole mass is in reaction, the molten alumina floating above the iron is cast into the form  $f f'$ . This alumina-slag congeals at once upon the cold surfaces of the rails and the bottom as well as the side walls of the mold and forms coatings  $d i$ , which protect the top part of the rails against getting deformed. The other part of the alumina-slag between the coatings is still liquid, but congeals also by and by. Then the iron is cast into the mold  $b'$  after a hole  $o$  has been punched through the bottom of the mold  $b$  and the alumina coating  $i$ . Evidently the bottom of the mold  $b$  will not offer great resistance to punching the hole through, since the metal has been heated by the alumina.

As already mentioned, the alumina has the purpose to heat the two parts to be welded together, while the iron shall form a rail-fish around the bottom parts of the two rails in order to strengthen the joint. The two rails are pressed together after the molten mass has been cast into the molds, so that a sufficient heat has been delivered to the parts to be welded. According to tests it has been found that one and one-half minutes suffice for heating the rails sufficiently for welding the same.

After the process has been carried out in the above-described way the molds are taken off and the alumina coating is knocked off, so that a rail is obtained, as shown in Fig. 3, in which figure  $a^2$  is the rail-fish, and  $g$  is a knob formed in  $o$  by the overflowing metal, which knob is afterward also knocked off.

In the modification shown in Fig. 4 two separate openings  $e e'$  for the alumina and the iron are provided. Through the opening  $e$  the alumina and through  $e'$  the molten iron is cast into the molds. The process is carried out in the same way as described above.

In Fig. 5 a mold is shown consisting of two parts separated in line  $m m$ , so that on one side  $r$  of the rails the alumina and on the other side  $r'$  of the rails the iron is cast. The rail-fish  $t$  would be arranged in this case only on one side of the rails and would extend to a certain height  $g'$ .

The process may be carried out also in another way. The top mold in Fig. 1 might be enlarged so as to receive the whole mass, consisting of the molten alumina and the iron. Then a hole is punched through the bottom

of this mold, whereby the molten iron flows through this hole around the lower part of the rails.

Another form of arrangement is shown in Fig. 6, in which the two molds are not arranged one above the other, but one mold  $x$  at the side of the other one  $y$ , the molds not touching each other, but being perfectly separated and leaving a space of about one-half inch between the same. Into this free space  $z$  between the two molds the molten iron is cast up to a certain height  $h$ , whereas in the two molds the liquid alumina is cast. The heating of the welding-face will be obtained by the conduction of the heat transferred to the rails by the alumina.

The most practical form of carrying the process into effect is illustrated in Figs. 7, 8, 85 and 9. In these figures 1 is a mold. 2 is a crucible situated above the same and provided with a tap-hole 3, which tap-hole may be closed by means of a plug or, as shown in the drawings, by means of a plate 10, consisting of sheet-iron, asbestos, or the like. 6 is the reaction mass. 4 are the rails to be joined. As will be seen from the drawings, the crucible is situated so that the tap-hole 3 is not situated vertically above the head of the rail. 95 If the reaction mass 6 is ignited, the highly-overheated metal 7, Fig. 8, melts the plate 10 and flows into the space 5 of the mold 1 and from there around the foot of the rail, as may be seen from the drawings, the alumina 8 flowing out after the metal flows around the upper part of the rail, as will be seen from Fig. 9. It will be understood that instead of arranging a special crucible above the mold this mold may be provided with a funnel 12 105 on its top, in which funnel the mixture can be filled.

Contrary to the known process consisting in casting metals around the lower part of the rails by the process described above a better 110 welding or joining of the metal cast around the rail-foot with this rail-foot is attained by the high superheat of the metal, whereby it is attained that the joining faces are joined in that way that one continuous metal piece is 115 formed.

Having thus fully described the nature of my said invention, what I desire to secure by Letters Patent of the United States is—

1. Process of joining metals by means of the 120 heat arising by the reaction taking place when pulverized aluminium and oxygen containing metal compounds are mixed and this mixture is ignited, said process consisting in casting the highly-overheated molten metal arising 125 by the reaction directly around one part of the metal pieces to be joined, and the molten alumina around another part of these metal pieces, substantially as described and for the purpose set forth.

2. Process of joining metal pieces, consisting in surrounding the ends to be joined with the mold, filling this mold partly with highly-overheated molten metal and partly with mol-

ten alumina substantially as described and for the purpose set forth.

3. Process of joining metal pieces consisting in surrounding the ends to be joined with a mold filling a crucible provided with a tap-hole in the bottom, with a mixture consisting of aluminium and an oxygen-containing metal compound, bringing the crucible above the mold in that way that the tap-hole is not situated vertically above the parts to be joined, igniting the mixture contained in the crucible and opening the tap-hole of the same, substantially as described and for the purpose set forth.
- 15 4. Process of joining metal pieces consisting in surrounding the ends to be joined with a mold filling a crucible provided with a tap-hole in the bottom, with a mixture consist-

ing of aluminium and an oxygen-containing metal compound, after the tap-hole being closed by means of a substance capable of being molten by the heat arising by the reaction taking place by the ignition of the mixture mentioned above, bringing the crucible above the mold in that way that the tap-hole is not situated vertically above the metal pieces to be joined and igniting the mixture contained in the crucible, substantially as described and for the purpose set forth.

In testimony whereof I have signed my name to this specification in the presence of two subscribing witnesses.

HANS GOLDSCHMIDT.

Witnesses:

WILLIAM ESENWEIN,  
PETER LIEBER.